

## UNITED STATES PATENT OFFICE

2,346,295

## CORROSION INHIBITION

Hans C. Duus, Wilmington, Del., assignor to E. I.  
du Pont de Nemours & Company, Wilmington,  
Del., a corporation of Delaware

No Drawing. Application November 12, 1941,  
Serial No. 418,699

20 Claims. (Cl. 252—74)

This invention relates to the prevention of corrosion and more particularly to prevention of corrosion in presence of alcohols and alcohol-containing antifreeze compositions.

Many different substances have previously been proposed for use as freezing point depressants in cooling fluids and among such suggested materials various mono- and polyhydric alcohols, alone or in combination, have been widely accepted.

In the use of such different freezing point depressants, particularly in connection with the cooling systems of internal combustion engines, various problems of corrosion have developed due, primarily, to the wide variety of metals and alloys with which water and the antifreeze liquids come in contact and against which metals there are exerted varying degrees of corrosion. Consequently, along with suggestions for use of such different freezing point depressants, there have been recommendations for employing as many, if not a greater number of, substances which are active for inhibiting corrosion of metals with which the water and freezing point depressants come in contact.

The practical disadvantages of prior corrosion inhibitors have been high cost or slight efficiency or both. Furthermore, the majority of previously proposed corrosion inhibitors have had little or no effect upon the corrosion caused by the alcohols upon the inner walls of the containers in which antifreeze liquids are normally packaged and stored.

It is an object of this invention to provide a new and improved class of corrosion inhibitors for use with alcoholic antifreeze materials. Other objects and advantages of this invention will be apparent hereinafter.

I have found that water soluble, normally liquid aliphatic mono- or polyhydric alcohols such, specifically, as methanol, ethanol, the propanols, butanols, ethylene glycol, and propylene glycol, the butylene glycols and glycerine, may be inhibited in their normally corrosive action upon the metal parts with which they come in contact, whether the metal parts are contained within the cooling system of an internal combustion engine or comprise the containers within which such antifreeze liquids are normally packaged and stored. For example, in the use of terne-plated cans, particularly when the plated surfaces thereof are in contact with glycol or glycol-containing solutions, no staining or corrosion of the surfaces is apparent when the inhibitors of this invention are present and dilution of the glycol with water causes no formation of undesirable white precipi-

tates such as are normally apparent in the absence of my corrosion inhibitor. These advantages and novel effects may be obtained, according to this invention, by adding to monohydric or polyhydric alcohols such as methanol, ethanol, ethylene glycol, propylene glycol, or the like, relatively small quantities of a carbonate having the formula  $XR\text{CO}_3$ , in which X represents an alkali metal and R represents an alkyl or hydroxy alkyl radical such as  $\text{CH}_2\text{CH}_2\text{OH}$  (the hydroxy alkyl radical of ethylene glycol) or  $\text{CH}_2\text{CHOHCH}_2\text{OH}$  (the hydroxy alkyl radical of glycerine). Thus, according to the present invention, I have found that the corrosive effect of mono- or polyhydric alcohols may be avoided by the addition thereto of from 0.01 to 5% by weight, based upon the alcohol, of such specific carbonates as sodium or potassium alkyl carbonates or sodium or potassium glycol carbonates.

Although larger and smaller quantities may be used effectively, if desired, I have found that 0.2 to 2.0% of the carbonate, based upon the weight of the alcohol, is preferred, with 0.2 to 1.0% being usually sufficient, to inhibit attack by the alcohol upon metals such as iron, copper, brass, solder and tin which are found in the metal parts of cooling systems of internal combustion engines or in the containers within which alcohols are normally packaged or stored.

The carbonates of the present invention may be added to the alcohol in any manner desired, such as by first mixing with a small quantity of alcohol, in order to obtain a homogeneous alcohol-carbonate solution, and the carbonate-containing alcohol thereafter mixed with larger quantities of alcohol or, alternatively, the carbonate may be produced directly in the main body of alcohol which is to be treated. If the latter procedure is preferred, it may be accomplished by adding the desired amount of an alkali metal hydroxide to the alcohol to be treated and thereafter bubbling carbon dioxide through the resulting mixture until neutrality is reached as shown by phenolphthalein.

As an example, 0.4 gram of alkali metal hydroxide may be added to each 100 cc. of alcohol and thereafter carbon dioxide bubbled therethrough until neutrality is reached. In such a case approximately 0.44 gram of carbon dioxide will be added per 0.4 gram of alkali metal hydroxide.

Various changes may be made in the methods and preferred embodiments of this invention without departing therefrom or sacrificing any of the advantages thereof.

I claim:

1. A method for inhibiting corrosion of metals in contact with normally liquid aliphatic alcohols which comprises incorporating in the alcohol, based upon the weight of the alcohol, from 0.01 to 5% of a carbonate having the general formula  $XRCO_3$ , in which X represents an alkali metal and R represents a radical selected from the group consisting of alkyl and hydroxy alkyl radicals.
  2. A method for inhibiting corrosion of metals in contact with normally liquid aliphatic alcohols which comprises incorporating in the alcohol, based upon the weight of the alcohol, from 0.2 to 2.0% of a carbonate having the general formula  $XRCO_3$ , in which X represents an alkali metal and R represents a radical selected from the group consisting of alkyl and hydroxy alkyl radicals.
  3. A method for inhibiting corrosion of metals in contact with normally liquid aliphatic alcohols which comprises incorporating in the alcohol, based upon the weight of the alcohol, from 0.01 to 5% of sodium methyl carbonate.
  4. A method for inhibiting corrosion of metals in contact with normally liquid aliphatic alcohols which comprises incorporating in the alcohol, based upon the weight of the alcohol, from 0.2 to 2% of sodium methyl carbonate.
  5. A method for inhibiting corrosion of metals in contact with normally liquid aliphatic alcohols which comprises incorporating in the alcohol, based upon the weight of the alcohol, from 0.01 to 5% of sodium glycol carbonate.
  6. A method for inhibiting corrosion of metals in contact with normally liquid aliphatic alcohols which comprises incorporating in the alcohol, based upon the weight of the alcohol, from 0.2 to 2% of sodium glycol carbonate.
  7. A method for inhibiting corrosion of metals in contact with normally liquid aliphatic alcohols which comprises adding to the alcohol from 0.2% to 1.0%, based upon the weight of the alcohol, of an alkali metal hydroxide and thereafter passing carbon dioxide into the alcohol until neutrality is reached.
  8. A method for inhibiting corrosion of metals in contact with normally liquid aliphatic alcohols which comprises adding to the alcohol from 0.2 to 1.0%, based upon the weight of the alcohol, of sodium hydroxide and thereafter passing carbon dioxide into the alcohol until neutrality is reached.
9. A method for inhibiting corrosion of metals in contact with methanol which comprises adding to the alcohol from 0.2 to 2% of an alkali metal alkyl carbonate.
10. A method for inhibiting corrosion of metals in contact with ethylene glycol which comprises incorporating in the glycol from 0.2 to 2% of an alkali metal hydroxy alkyl carbonate.
11. A method for inhibiting corrosion of metals in contact with methanol which comprises adding to the alcohol from 0.2 to 2% of sodium methyl carbonate.
12. A method for inhibiting corrosion of metals in contact with ethylene glycol which comprises incorporating in the glycol from 0.2 to 2% of sodium glycol carbonate.
13. An antifreeze composition consisting substantially entirely of a normally liquid aliphatic alcohol containing from 0.01 to 5% of a carbonate having the general formula  $XRCO_3$ , in which X represents an alkali metal and R represents a radical selected from the group consisting of alkyl and hydroxy alkyl radicals.
14. An antifreeze composition consisting substantially entirely of a normally liquid aliphatic alcohol containing from 0.2 to 2% of a carbonate having the general formula  $XRCO_3$ , in which X represents an alkali metal and R represents a radical selected from the group consisting of alkyl and hydroxy alkyl radicals.
15. An antifreeze composition consisting substantially entirely of methanol containing from 0.01 to 5% of an alkali metal alkyl carbonate.
16. An antifreeze composition consisting substantially entirely of methanol containing from 0.01 to 5% of an alkali metal methyl carbonate.
17. An antifreeze composition consisting substantially entirely of methanol containing from 0.01 to 5% of sodium methyl carbonate.
18. An antifreeze composition consisting substantially entirely of ethylene glycol and from 0.01 to 5% of an alkali metal hydroxy alkyl carbonate.
19. An antifreeze composition consisting substantially entirely of ethylene glycol and from 0.01 to 5% of an alkali metal glycol carbonate.
20. An antifreeze composition consisting substantially entirely of ethylene glycol and from 0.01 to 5% of sodium glycol carbonate.